

Sept. 2, 1952

L. K. CHENEY

2,609,331

PYROLYTIC CONVERSION OF OIL SHALE

Filed June 17, 1947



BY

LEROY K. CHENEY

ATTORNEYS

*Penick, Edwards, Morton Barrows*

## UNITED STATES PATENT OFFICE

2,609,331

## PYROLYTIC CONVERSION OF OIL SHALE

Leroy K. Cheney, Lansing, Ill., assignor to Sinclair Refining Company, New York, N. Y., a corporation of Maine

Application June 17, 1947, Serial No. 755,231

3 Claims. (Cl. 202—11)

1

This invention relates to improvements in the recovery of oil from oil-bearing shale and more particularly to the process of producing shale oil from oil-bearing shales by the thermal pyrolysis thereof in the presence of a catalyst which favors the disintegration of the shale and the production of oil therefrom.

Many proposals have been made over a long period of years for the recovery of oil from oil-bearing shales, but because of economic reasons American shales have not been worked on a commercial scale. As long as the price of petroleum oil was low enough and it was sufficiently plentiful, it was impracticable to produce shale oil in competition. However, the natural resources of petroleum are being used up at an enormous rate and costs of petroleum production are increasing. The recovery of oil from oil shale therefore becomes more practical and necessary.

An important feature of my invention relates to the retorting of oil shale in the presence of catalysts which permit the use of lower retorting temperatures and produce improved shale oil products of higher API gravity.

In accordance with features of my invention I advantageously grind the oil shale to be retorted in water to form a slurry, and treat this slurry with an acid so as to change some of the inorganic constituents of the shale into active catalytic form. The resulting mixture is then filtered, dried and retorted.

My improved process includes other features, objects and advantages, as pointed out hereinbelow in connection with the accompanying drawing forming a part of this application.

In the drawing, the single figure is a diagrammatic view partly in elevation, illustrating an apparatus in which the steps of my improved process may be carried out.

The oil shale to be processed, in an advantageous form of my invention, is introduced into the apparatus from a suitable supply through a chute or conduit 2, provided with a rotary feed valve 4, into a crusher or grinder 6 which may be of any suitable type, the grinding elements of which may be operated by a drive-wheel 8. The process may be operated in a continuous manner or in batch or in semi-batch procedure, but is illustrated by the grinding of a suitable quantity of shale in the grinder 6 in the presence of water introduced through a valved line 10 so as to produce a slurry. During the final stages of grinding of the slurry, a catalytic acid such as hydrofluoric acid or hydrochloric acid, is introduced into the grinder 6 through a line 12, and intimately mixed and ground with the slurry. The proportion of

2

acid to oil shale may vary from 0.5 to 6% of the dry shale by weight, depending upon the pH of the slurry and the acid used.

The other parts of the apparatus shown below the grinder 6 includes a mixer 14 and a filter 16. The mixture of slurry and catalyst produced in the grinder 6 is preferably conducted through a conduit 20, having a rotary feed valve or other type of valve therein so that the completion of the mixing operation is effected in the mixer 14, which may be operated, for example, by a drive-wheel 22. A new batch may then be started in the grinder 6.

After the mixing is completed, the oil shale and catalyst or activated slurry form is conducted through a conduit 24, having a rotary feed valve or other type of valve therein, into the filter 16. Any solution removed by the filter is withdrawn therefrom through a valved line 26, and thereafter the filter cake, which of course is still wet, is dried and therefore preferably conveyed directly into a dryer 28 from the filter 16, as for example, through a chute, conveyor or conduit, illustrated by the conduit 30, having a rotary feed valve or other type valve therein. In the operation described, the wet catalytically active oil shale is dried in any suitable manner in the dryer 28, the moisture-laden air produced by the drying being withdrawn through a flue 32.

The dryer 28 may be of any conventional form, as for example, a continuous belt or chain dryer provided with means for supplying heat and air for drying purposes. The dried catalyst and finely ground oil shale is transferred from the dryer 28 through a sealing rotary feed valve 34 into a retort 36 where the catalyzed oil shale is retorted at a suitable temperature of from 850° F. to 1100° F. for the production and recovery of oil from the shale. The spent shale is discharged from the retort through a chute 38 provided with a sealing rotary feed valve, as indicated.

The oil vapors produced in the retorting operation are conducted through a vapor line 40 into a fractionating tower 42 in which the higher boiling constituents of the oil, as for example, that boiling above the gasoline range, is condensed, the resulting condensed product being withdrawn through a valved line 44. The gases and gasoline constituents produced in the retorting operation are conducted overhead from the tower 42 through a vapor line 46 and subjected to cooling and condensation in a condenser 48. The condensate and gases are withdrawn through a valved line 50 to a suitable gas separator and condensate receiver (not shown).

The retort 36 may be of any conventional type

such as an inclined retort in which the shale is fed gradually therethrough and subjected to heat produced in the lower part 52 of the retort, which may include suitable burners and combustion chambers. Other types of retorts may be used, such as vertical or inclined gravity feed retorts in which means is provided for removing vapors at points adjacent their formation. The retort 36, as shown, may be provided with a conveyor means by which the oil shale is slowly moved through the retort while it is being heated to produce the shale oil.

The acid used in the pretreatment of the shale during the grinding and mixing operations, reacts with the inorganic constituents in the shale, such as the silicon, aluminum and iron compounds to produce active catalysts which greatly facilitate the production of the oil from the shale with a minimum of carbon production, and at the same time produce a shale oil product which has a higher API gravity than would otherwise be produced. During the retorting operation under catalytic conditions, the oil at the instant it is produced from the shale also comes under the influence of the catalyst at the high temperatures necessary, and is to a considerable extent, converted to products of lower API gravity so that in a retorting operation as described, a considerable proportion of the oil product is gasoline range material of acceptable anti-knock value, particularly high in aromatic hydrocarbons when compared to the usual type of product.

The aluminum halide catalysts are particularly effective for improving the recovery of oil from oil shale. For example, aluminum chloride, aluminum fluoride, or mixed aluminum chlorides and fluoride, or complex aluminum fluorochlorides. Any known oil cracking catalyst may be used in my process in addition to those mentioned above, and mixtures of catalysts may be employed, as for example, hydrogen fluoride or hydrochloric acid may be used along with the catalyst salts or oxides. Acid mixed with the catalyst slurry in the grinder 6 and mixer 14 is adsorbed into the oil shale to produce complex catalytic materials with the constituents of the shale.

I claim:

1. In the process of producing shale oil from oil shale, including the retorting of the oil shale, the improvement which comprises grinding the oil shale to be processed with water to form a slurry, treating the slurry with a material selected from the group consisting of hydrochloric acid, hydrofluoric acid, and hydrogen fluoride in an amount equal to 0.5 to 6% by weight of the oil shale in the slurry while thoroughly mixing

said material with the slurry thereby catalytically activating inorganic constituents of the oil shale, filtering the slurry to remove excess water, drying the filtered oil shale, and subjecting it to a retorting operation and producing shale oil therefrom.

2. In the process of producing shale oil from oil shale, including the retorting of the oil shale, the improvement which comprises grinding the oil shale to be processed with water to form a slurry, treating the slurry with hydrofluoric acid in an amount equal to 0.5 to 6% by weight of the oil shale in the slurry while thoroughly mixing said material with the slurry thereby producing a fluoride catalyst for catalyzing the shale oil production in the retorting operation, filtering the slurry to remove excess water, drying the filtered oil shale, and subjecting it to a retorting operation and producing shale oil therefrom.

3. In the process of producing shale oil from oil shale, including the retorting of the oil shale, the improvement which comprises grinding the oil shale to be processed with water to form a slurry, treating the slurry with hydrogen fluoride in an amount equal to 0.5 to 6% by weight of the oil shale in the slurry while thoroughly mixing said material with the slurry thereby producing a fluoride catalyst for catalyzing the shale oil production in the retorting operation, filtering the slurry to remove excess water, drying the filtered oil shale, and subjecting it to a retorting operation and producing shale oil therefrom.

LEROY K. CHENEY.

#### REFERENCES CITED

The following references are of record in the file of this patent:

#### UNITED STATES PATENTS

| Number    | Name          | Date          |
|-----------|---------------|---------------|
| 1,276,879 | Crane         | Aug. 27, 1918 |
| 1,280,178 | Day           | Oct. 1, 1918  |
| 1,510,983 | Dolbear       | Oct. 7, 1924  |
| 1,773,339 | Zieley et al. | Aug. 26, 1930 |
| 1,941,809 | McKee         | Jan. 2, 1934  |
| 2,431,677 | Brown         | Dec. 2, 1947  |

#### FOREIGN PATENTS

| Number            | Country       | Date           |
|-------------------|---------------|----------------|
| 290,606           | Great Britain | Apr. 25, 1929  |
| 394,639           | Great Britain | Sept. 21, 1931 |
| 19,231<br>of 1934 | Australia     | Sept. 5, 1935  |

#### OTHER REFERENCES

Bureau of Mines Information Circular 7481, October 1948, pages 8 to 11 and Figure 3.